

2,954,387

## FATTY ACID COMPOUNDS FOR USE AS DRYING OILS

Herman S. Bloch, Skokie, Ill., assignor, by mesne assignments, to Universal Oil Products Company, Des Plaines, Ill., a corporation of Delaware

No Drawing. Filed Oct. 5, 1955, Ser. No. 538,777

9 Claims. (Cl. 260—407)

This invention relates to a process for treating fatty acid compounds, and particularly fatty acid glycerides, for increasing unsaturation between the carbon bonds in said compounds and/or for isomerizing the unsaturated linkages in such compounds to a more highly conjugated system of ethylenic bonds. More specifically, the present invention concerns a process for effecting isomerization and/or dehydroisomerization of fatty acid compounds selected from the fatty acids themselves, their salts, esters, and amides to produce thereby compounds in which the unsaturated bonds are in conjugated relationship with each other.

One object of the invention is to enhance the air-drying properties of unsaturated fatty acid compounds. Still another object of the invention is to improve the chemical reactivity of the present fatty acid compounds and thereby enhance their value as starting materials in the production of derivatives thereof and to convert fatty acid compounds having inferior properties of little or no utility to superior products which may be readily utilized in various syntheses and for various commercial uses.

In one of its embodiments the present invention relates to a process for isomerizing a fatty acid compound to a product having a conjugated system of unsaturated linkages which comprises contacting said fatty acid compound at an elevated temperature with an alkaline metal addition complex of an organic compound in which the metal is bonded to the organic compound through a metal-carbon atom linkage.

A more specific embodiment of the invention concerns the isomerization of linseed oil to a product having enhanced drying properties in which the unsaturated linkages have a more highly conjugated relationship with respect to each other by contacting said linseed oil with an alkali metal-hydrocarbon addition complex at a temperature of from about 100° to about 300° C., at a pressure sufficient to maintain the reaction mixture in substantially liquid phase and for a time sufficient to effect such isomerization.

A more specific embodiment of the invention concerns the dehydroisomerization of soybean oil whereby a product having enhanced drying properties is formed, in which process said soybean oil is contacted at a temperature of from about 150° to about 300° C. with a mixture of a sodium-alkyl catalyst and a promoter consisting of anthracene, utilizing an inert gaseous atmosphere, at a pressure sufficient to maintain the reaction mixture in substantially liquid phase.

It is well-known that many fatty acid ester oils of naturally occurring origin have widely different drying properties when exposed to atmospheric oxygen. Thus, many oils such as soybean oil and sunflower oil dry very slowly, if at all, when exposed to atmospheric drying conditions and are therefore generally considered non-drying or semi-drying oils, although they exist in abundance and would normally find wide usage if they possessed better drying qualities and greater chemical reactivity. Other naturally occurring oils of the fatty acid glyceride

type dry upon exposure to atmospheric oxygen only after relatively prolonged periods of time or with the addition of so-called "driers" which promote the speed of the drying reactions, including such oils as linseed oil, dehydrated castor oil, and others belonging to this class. Still other oils of natural origin dry upon exposure to atmospheric oxygen at relatively high speeds, but their source of supply is relatively limited and they are consequently relatively expensive and in short supply, including such oils as tung oil and oiticica oil. In many instances the fatty acids and certain fatty acid derivatives, such as the esters of the lower molecular weight alcohols of monohydric, dihydric and trihydric classes and the amide derivatives would be of considerably greater economic importance were a method available for converting such fatty acid compounds into more highly unsaturated derivatives thereof and particularly derivatives in which the unsaturation is of the conjugated variety. The present invention is primarily concerned with the conversion of fatty acids, fatty acid salts, fatty acid esters and fatty acid amides into their more highly unsaturated derivatives and particularly such derivatives in which the unsaturated linkages become arranged in conjugated relationship to each other. The means herein provided for effecting such conversion comprises contacting the fatty acid compound with an alkaline earth or alkali metal-hydrocarbon addition complex at reaction conditions which effect the isomerization and/or dehydroisomerization of the fatty acid compound to a product containing a greater number of unsaturated linkages and/or a product in which the unsaturated linkages are in conjugated relationship with each other. In certain instances, it has been found desirable to incorporate into the reaction mixture an organic compound hereinafter more specifically characterized, having a promoting effect on the isomerization and/or dehydroisomerization reaction, in order to increase the yield of isomerized product and/or the rate of the resulting isomerization or dehydroisomerization reaction.

The starting materials or charging stocks utilizable in the present process may be selected from the drying, semi-drying, or the essentially non-drying types of naturally occurring oils which exist in their natural state as glycerides and these may be of vegetable, animal or marine origin. Although naturally occurring fatty acid glycerides provide a convenient source of starting materials, it may be preferred in certain cases to utilize other alcohol esters of the fatty acid portion of the oil, for example, the esters formed by replacing the glyceride ester linkage with other mono- or polyhydric alcohols, if desired. Thus, the naturally occurring oils may be hydrolyzed to free the fatty acid and the separated acid esterified with such alcohols as methanol, ethanol, isopropanol, a polyhydroxy alcohol such as ethylene glycol, pentaerythritol, sorbitol and the like or an alkanolamine, represented, for example, by the mono- and polyethanolamines. Instead of esterifying these released fatty acids, they may also be reacted with certain alkaline bases, such as sodium, potassium or lithium hydroxide, calcium, magnesium or barium hydroxide, their carbonates, bicarbonates or weak acid salts or with other metal hydroxides to form the corresponding soaps and the latter utilized in the present process as charging stock. These soaps may also be prepared by direct hydrolysis and neutralization of the fatty acid glyceride, forming a soap in situ. In certain other instances the amide derivatives of the fatty acids may be the preferred starting materials in the present process, including the fatty acid amides of ammonia and such amines as methylamine or dimethylamine, mono- or diethylamine, a polyamine, such as ethylene diamine, diethylene triamine, triethylene tetra-amine, an aromatic amine such as aniline

or other amide products formed by dehydration of the fatty acid amine salt.

Typical fatty acid oils which illustrate the type of fatty acid glycerides utilizable in the present process are such drying and semi-drying types as linseed oil (either raw or boiled linseed oil), castor oil or dehydrated castor oil, perilla oil, olive oil, peanut oil, walnut oil, cottonseed oil, cocoanut oil, soybean oil, hempseed oil, poppyseed oil, safflower oil, sunflower seed oil, whale oil, menhaden oil, lard, tallow and other well-known fatty acid glycerides. The fatty acids, when preferred herein, may be prepared from the naturally occurring oil by hydrolyzing the oil, for example by caustic, followed by acidification of the resulting soap and recovery of the released fatty acid. Although it is generally preferred to employ fatty acid compounds initially containing at least 1 double bond per molecule, great economic advantages may be obtained in dehydroisomerizing a normally saturated or only partly unsaturated fatty acid compound in order to convert a material having little initial value as a drying oil into a product of substantially greater drying properties by the present dehydroisomerizing process in which unsaturated bonds in conjugated relationship may be introduced into the compound and the resulting product thereby enhanced in value. Still another class of materials utilizable as the initial charging stock may be the oil-modified alkyd resins, oil-modified phenolic, or other drying oil-modified resinous materials prepared in a preceding synthesis.

The isomerization and dehydroisomerization reactions, herein referred to generically as isomerization processes are effected in accordance with the present invention by contacting the above-indicated starting material with an alkaline earth or alkali metal-addition complex of certain organic compounds which combine with the alkaline earth or alkali metal through a metal-carbon atom bond to form an active isomerization or dehydroisomerization catalyst, the particular resulting reaction depending upon the temperature and other conditions maintained during the conversion. These catalysts are usually prepared prior to the isomerization process of this invention within the reaction vessel in which the isomerization is effected by combining an alkali metal such as sodium, potassium, lithium, rubidium and cesium or an alkaline earth metal, such as beryllium, magnesium, calcium, strontium or barium with an organic compound and particularly a hydrocarbon compound containing an active hydrogen atom on one of the carbon atoms of the compound which reacts with the metal to form a metal-carbon atom bond. Such hydrocarbons include the branched chain aliphatic hydrocarbons, such as isopentane, 2,3-dimethylbutane, 2,4-dimethylpentane, 2,2,3 - trimethylbutane, 2,3,4 - trimethylpentane and other homologous hydrocarbons containing up to about 12 carbon atoms per molecule. Other hydrocarbons suitable for forming the alkaline earth or alkali metal-hydrocarbon addition complexes are the aromatic hydrocarbons, including benzene, toluene, xylene, mesitylene, cumene, naphthalene, anthracene, fluorene, tetralin, dihydronaphthalene, dihydroanthracene, phenanthrene and their halogen-substituted derivatives such as chlorobenzene, o-chlorotoluene, p-bromoxylene, o-chloropropylbenzene, etc.; the alkyl-substituted and particularly methyl-substituted derivatives of the above such as dimethyl naphthalene, mono-, di-, and triphenyl methane; and hydrocarbons containing an acetylenic linkage, such as acetylene itself, propyne, ethylacetylene, pentyne, hexyne, heptyne, and higher homologs. Of the above, it is generally preferred to utilize the sodium and potassium-hydrocarbon addition complexes and of these, the complexes thereof with aromatic hydrocarbons such as naphthalene, toluene, cumene and the complex thereof with acetylene are generally preferred because of their high order of effectiveness in accomplishing the desired isomerization and dehydroisomerization reactions herein provided. The catalyst comprising the alkaline metal-hydrocarbon addition complexes may be charged individ-

ually into the reaction mixture as the complex itself or separately to form the alkaline metal-hydrocarbon addition complex in situ during the ensuing reaction, or the catalyst complex as such may be deposited upon or supported by an inert refractory substance, preferably selected from the refractory metal oxides, such as alumina, silica, magnesia, or upon other types of supporting materials such as coke, charcoal, pumice, quartz, iron turnings, copper shot, ceramic saddles, etc.

10 The isomerization and dehydroisomerization reactions of the present invention are promoted by the addition of a small amount of a compound which is capable of forming a free radical in the presence of the catalyst and reactants and during the course of the isomerization reaction. 15 These compounds, referred to herein as "promoters" by virtue of their catalyzing properties in either increasing the yield of isomerized product or in increasing the rate of the isomerization reaction combine with the alkaline metal to form a carbon-metal bond. Compounds of this 20 character include heterocyclic compounds containing nitrogen in the nucleus of the ring such as pyridine, picoline, quinoline, isoquinoline, pyrrole, piperidine, and their nucleophilic alkylated derivatives; organic peroxide compounds such as acetyl peroxide, benzoyl peroxide, di-butyl peroxide, t-butyl hydroperoxide, tetrinaline hydroperoxide, methylcyclopentyl hydroperoxide, dimethylcyclopentyl hydroperoxide, cumene hydroperoxide and others. Other organic-metalloc compounds in which the 25 organic radical is attached to the metal through a carbon-metal bond may also be utilized as promoters in the present process, including such compounds as the lead tetra-alkyls, such as tetra-ethyl lead, a lead tetra-aryl, a lead alkylaryl, a zinc aryl, certain mercury dialkyls and diaryls, tin tetra-alkyls, and other organometallic compounds.

30 The amount of alkaline metal (i.e., alkaline earth or alkali metal) required and the amount of organic promoter preferred for use in the isomerization reaction are dependent upon the reaction conditions and upon the particular fatty acid compound charged to the process. 35 In general, an excess of the alkaline metal over the organic compound capable of forming the organometallic complex utilized as the catalyst is employed in the reaction, thereby ensuring the presence of free metal in the reaction zone, above that required to form the organometallic complex and to provide from 0.1 to about 20% by weight thereof based on the fatty acid compound charged to the reaction zone, the ultimate proportion required in many particular instances depending upon the depth of the dehydroisomerization of the charging stock desired. Since the catalyst is substantially unaltered during the course of the process, the catalyst may be recovered from the reaction products and recycled, if desired, in a succeeding reaction with additional charging stock.

40 The process of this invention may be carried out in any suitable manner, including batch or continuous methods of operation, in an autoclave or a reaction vessel constructed of tubes through which the reactants are continuously charged, the latter being constructed either of steel or in the form of a glass-lined steel reactor. The 45 process is carried out by charging the fatty acid compound in admixture with the alkaline metal-hydrocarbon complex to which mixture the promoter is added, if desired, into the reaction zone maintained at a temperature of from about 100° to about 300° C., preferably at a temperature of from about 150° to about 275° C., sufficient pressure being applied to the reaction mixture to maintain the reactants in substantially liquid phase condition. Although not necessarily required, inert gas may be charged into the reactor to obtain the desired pressure which may range from atmospheric to 50 atmospheres, or more, in order to provide the above preferred liquid phase conditions. Such inert gases as nitrogen, carbon dioxide, methane, ethane, etc. also provide a blanket of inert atmosphere above the reactants to exclude oxygen from the system.

In a typical batch-type operation, a quantity of the fatty acid compound and catalyst comprising the alkaline earth or alkali metal, the corresponding metal-hydrocarbon complex or a mixture of the metal and an organic promoter is placed in the reactor which is preferably equipped with a suitable mixing device to maintain the catalyst, promoter and fatty acid compound in intimate contact with each other during the reaction. The mixture of reaction products, catalyst and promoter, following the completion of the isomerization reaction, is thereafter subjected to a suitable separation procedure, as for example, decantation or filtration, to recover unconsumed catalyst, followed by fractional distillation of the organic product to separate the promoter from the desired isomerized fatty acid compound. As indicated previously, the catalyst thus separated may be recycled, if desired, to the isomerization reactor for repeated reuse therein.

It has been found that the isomerization of the fatty acid compound involving a shift in the position of the unsaturated linkages present in the charging stock to conjugated positions occurs at relatively lower temperatures within the temperature range above specified, generally at temperatures within the range of from about 100° to about 250° C. and with smaller amounts of catalyst and promoter than is required to effect dehydroisomerization of the fatty acid compound, the latter reaction in which more highly unsaturated fatty acid compounds are produced generally occurring at temperatures within the range of from about 150° to about 300° C. For the latter dehydroisomerization type of reaction, catalyst to charging stock ratios sufficient to provide from about 5% to about 20% of the alkaline metal in the reaction mixture, based upon the fatty acid compound charged, are preferably employed. It has also been found that the residence time of the catalyst within the reaction mixture, which, in general, may be within the range of from about one-half to about 6 hours, is usually greater for effecting dehydroisomerization than isomerization of the charging stock. In continuous types of operation, the residence time is measured as the average length of time the charging stock is within the reaction zone, maintained at the above temperature and pressure conditions, in contact with the catalyst. For the isomerization type of reaction, the residence time or period of contact between the charging stock and catalyst may be from about one-half to about 3 hours, while dehydroisomerization is preferably effected over a reaction period of from about 2 to about 6 hours, more or less, depending upon the degree of saturation of the charging stock and the degree of unsaturation desired in the product.

Following completion of the isomerization or dehydroisomerization reaction the product is separated from the catalyst, usually by merely decanting the liquid product from the solid catalyst phase, thereafter washed with water to remove any dissolved or suspended catalyst and distilled, if necessary, to remove the promoter compound, if initially charged to the reaction mixture.

The present invention is further illustrated with respect to specific embodiments thereof in the following examples which, however, are not intended to limit the scope of the invention necessarily in accordance therewith.

#### Example I

A sample of linseed oil which normally dries at a relatively slow rate upon exposure to atmospheric oxygen to form a relatively soft, abrasion-responsive film, is converted by isomerization to a product which dries at the same drying conditions at a higher rate of speed and which produces, when dried, a harder, tougher dried film than the starting material in accordance with the process of the present invention by means of the following procedure.

20 weight proportions of sodium and 50 weight proportions of anthracene, previously dried by distillation, are mixed in a stirred reactor at 100° C. for 1/2 hour to form

a sodium-anthracene complex which exists in the form of a semi-solid form when cooled. To the above complex is added 1000 weight proportions of a previously dried linseed oil having an iodine number of 170 and a maleic anhydride value of 7, the linseed oil being added at room temperature. The autoclave is then flushed with nitrogen, thereafter sealed and then charged with nitrogen to 100 atmospheres pressure. The autoclave is then stirred by means of a rapidly rotating stirring pedal mounted on the inside of the autoclave as the latter is heated to a temperature of 175° C. for 3 hours, followed by cooling to room temperature. The isomerized linseed oil product is decanted from the solid phase within the reactor and heated to 200° C. at 0.5 mm. Hg pressure to distill over a major proportion of the dissolved anthracene. The recovered oil when tested for its drying properties by painting a thin film of the oil on a series of sheet aluminum test panels and after exposure to air at room temperature dries to a tack-free condition in approximately 10 hours and to a dried, hard film having a Sward hardness of 10 in approximately 1.5 days. The isomerized product has an iodine number of 197 and a maleic anhydride value of 20.

#### Example II

In the following run a sample of sunflower seed oil which has an iodine number of 130 and a maleic anhydride value of 8 is subjected to dehydroisomerization in accordance with the procedure described as follows:

This oil in its unmodified state, is substantially inert to atmospheric oxygen, a thin film of the oil sprayed on an aluminum test panel and exposed to air at room temperature remaining undried at the test conditions, even after exposure to the atmosphere over a period of 20 days.

The catalyst in the following run is sodium acetylide prepared by mixing in an autoclave 50 grams of metallic sodium in liquid ammonia and reacting the latter at a temperature of 50° C. with one equivalent of acetylene charged into the reactor at a pressure slightly in excess of 20 atmospheres. The reaction is assisted by stirring the liquid ammonia suspension of sodium with a high speed stirring paddle. The resulting sodium-acetylene addition product is a white solid after evaporation of the liquefied ammonia. To the resulting catalyst is added 1000 weight proportions of sunflower oil having the above drying characteristics, followed by flushing the system with nitrogen and charging nitrogen into the reactor to a pressure of 100 atmospheres. The contents of the reactor are thereafter stirred as the mixture is heated to a temperature of 300° C. for 6 hours. The reactor contents are then separated by decanting the liquid product from the solid catalyst and the recovered converted sunflower seed oil heated to drive off any dissolved acetylene. The recovered oil has an iodine number of 180, a maleic anhydride value of 22 and when tested for its drying properties by exposing a thin film of the oil on an aluminum test panel to air at room temperature it produces a tack-free film in less than 12 hours and dries to a film having a Sward hardness of 9 in approximately 38 hours.

I claim as my invention:

1. A process for improving the drying properties of glyceride oils which comprises heating the glyceride oil to a temperature of from about 100° to about 300° C. in the presence of an alkaline metal addition complex having a metal-carbon atom bond and in which the alkaline metal is complexed with a hydrocarbon selected from the group consisting of an acetylenic hydrocarbon and anthracene.
2. A process for improving the drying properties of glyceride oils which comprises heating the glyceride oil to a temperature of from about 100° to about 300° C. in the presence of an alkaline metal addition complex having a metal-carbon atom bond and in which the alkaline metal is complexed with an acetylenic hydrocarbon.
3. A process for improving the drying properties of glyceride oils which comprises heating the glyceride oil

to a temperature of from about 100° to about 300° C. in the presence of an alkaline metal addition complex having a metal-carbon atom bond and in which the alkaline metal is complexed with anthracene.

4. The process of claim 1 further characterized in that said glyceride oil is linseed oil.

5. The process of claim 1 further characterized in that said glyceride oil is sunflower oil.

6. The process of claim 1 further characterized in that the metal of said addition complex is sodium.

7. The process of claim 1 further characterized in that the alkali metal is complexed with an acetylenic hydrocarbon.

8. The process of claim 7 further characterized in that said complex is sodium acetylidyde.

9. A process for improving the drying properties of glyceride oils which comprises heating the glyceride oil to a temperature of from about 100° to about 300° C. in the presence of a sodium-anthracene complex.

References Cited in the file of this patent

UNITED STATES PATENTS

|    |           |                 |                |
|----|-----------|-----------------|----------------|
| 10 | 2,242,230 | Burr            | May 20, 1941   |
|    | 2,653,956 | Marhofer et al. | Sept. 29, 1953 |
|    | 2,740,820 | Wilson et al.   | Apr. 3, 1956   |